

# UNITED STATES PATENT OFFICE.

MARK W. MARSDEN, OF PHILADELPHIA, PENNSYLVANIA.

## TOBACCO WRAPPER AND PROCESS OF MAKING SAME.

SPECIFICATION forming part of Letters Patent No. 720,880, dated February 17, 1903.

Application filed April 17, 1902. Serial No. 103,406. (No specimens.)

*To all whom it may concern:*

Be it known that I, MARK W. MARSDEN, a citizen of the United States, residing at Logan Station, Philadelphia, in the county of Philadelphia and State of Pennsylvania, have invented a certain new and useful Improved Tobacco Wrapper and Process of Making the Same, of which the following is a specification.

10 The production from tobacco-stems and other tobacco waste of paper suitable for use as wrappers for cigars, cigarettes, and other purposes has been hitherto attempted or suggested, and although such a product is very 15 desirable and although many stems are practically wasted these attempts and suggestions have until now proven commercially unfruitful.

One object of the present invention is to 20 obviate the defects and disadvantages heretofore encountered and to provide a satisfactory and capable tobacco paper for such uses and also a method of making or preparing the same.

25 In the present invention the paper is made from the fibrous parts of the tobacco-stems freed from the cellular and extractive matter, and therefore is better than if the cellular matter were present, because it requires 30 no binder and is quite strong and is also better than if the extractive matter were present, because the latter contains potash, which is undesirable, and also an excess of saltpeter and also other noxious or undesirable materials. Moreover, in my invention the extractive matter is purified or freed from such 35 ingredients before its application to the paper, so that the taste, odor, quality, and way of burning the latter are unobjectionable.

40 To practice the invention, tobacco-stems in their natural condition—that is, without being comminuted—are subjected for two or three hours, more or less, to the action of steam at eighty pounds pressure, more or less, 45 and water. This may be accomplished in a closed vessel, such as a pulp-digester. The purpose of this is to loosen the cellular in respect to the fibrous tissue and to extract juice, saltpeter, potash, fusel-oil, tannin, and 50 other chemicals and matters, all of which, singly or collectively, with the exception of the cellular matter, are hereinafter referred

to by the term "extractive matter." The mass is further treated by straining to separate the cellular material and squeezing or 55 the like to eliminate the extractive as well as other matter, leaving substantially only the fibers. During this operation combing or rolling and washing may be resorted to, the purpose being, as stated, to obtain the fibers 60 freed from cellular matter and from extractive matter of an undesirable kind and in a good long and strong condition. The fibrous part may be treated by a repetition or repetitions of the described operation. The fibers 65 so treated are then pulped and made into paper—for example, by beating them up with water, as in a rotary beater, and forming them as on gauze or bringing them into sheet form, which sheets may be calendered, or, if 70 desired, embossed, to look like the markings of the natural leaf. If desired, from one to two per cent., by weight, of glycerin and from one-half per cent. to one per cent., by weight, of licorice may be added to the 75 pulp. The purpose of the glycerin is to improve its consistency or structure and of the licorice to flavor it. To color the paper and to add to it the qualities possessed by natural 80 tobacco-leaves, such as are used for wrappers, the pulp is impregnated or reinfused with a liquor prepared by treating the solution or juice derived from the boiling or digesting operation or operations. It is obvious that the same result would be accomplished by 85 staining or impregnating the paper itself. Some of the qualities referred to are an even retarded burning and the exhibiting of a grayish ash. For the purpose of reinfusing or impregnating the pulp or paper the extractive solution, from which the cellular and 90 solid matter may be strained, is heated under pressure in a closed receptacle to a temperature exceeding 250° Fahrenheit, so as to drive off fusel-oil and any other volatile constituent which will go off at that temperature. The pressure is then suddenly relieved and the fusel-oil and water blown over in the 95 form of steam or vapor. After the removal of the fusel-oil in the manner stated the extractive matter is usually left comparatively dry, and it may sometimes become necessary to add water to take the place of that which went over with the fusel-oil. Subse-

quently the extractive matter with the added water is evaporated, as by boiling, with the result that potash, some of the saltpeter, and other mineral matters crystallize out and are separated from the solution of liquor. The residue or purified extractive is then applied to the pulp solution above described, and it serves to stain and color the same, and also to flavor it, it being understood that there is sufficient water in the pulp to combine with the purified extractive and effect this purpose.

It will be obvious to those skilled in the art to which my invention appertains that modifications may be made in detail without departing from the spirit thereof. Hence I do not limit myself to the precise ingredients and mode of procedure hereinbefore set forth; but,

Having thus described the nature and objects of my invention, what I claim as new, and desire to secure by Letters Patent, is—

1. The process of making wrappers from tobacco stems and waste which consists in subjecting the stems and waste to heat and moisture to extract a solution of soluble juice and salts and to loosen the fibers and cellular matter, straining and pressing the mass to separate the fibers from the cellular matter and from the solution of soluble matter, making the separated fibers into pulp, extracting cellular and deleterious matter from the solution, and adding the resultant solution to the pulp, substantially as described.

2. An improved tobacco wrapper obtained from uncommunited tobacco fiber deprived of its cellular tissue, said fiber having an infusion of tobacco-juice from which objectionable matter has been eliminated.

3. The process of making wrappers from tobacco-stems and the like which consists in separating the cellular tissue and the extractive from the fibrous matter, making the fibrous matter into paper-pulp, purifying the extractive matter, and applying the purified extractive matter to the pulp, substantially as described.

4. The process of making wrappers from the fibrous portion of tobacco, which consists in first separating the cellular tissue and other deleterious matter from the fibers and then pulping and treating the fibers in the usual manner in paper manufacture, substantially as described.

5. The process of making wrappers from tobacco stems and waste, which consists in extracting the juice and separating the cellular tissue from the fiber, converting the fiber into pulp, and making the pulp into paper, substantially as described.

6. The process of making wrappers from tobacco stems and waste, which consists in separating the extractive and the cellular tissue from the fiber, converting the fiber into pulp, coloring the pulp and making it into paper, substantially as described.

7. The process of making wrappers from to-

bacco stems and waste, which consists in separating the extractive and the cellular tissue from the fiber, converting the fiber into pulp, flavoring the pulp, coloring it, and making it into paper, substantially as described.

8. The process of making wrappers from tobacco stems and waste, which consists in separating the extractive and the cellular tissue from the fiber, converting the fiber into pulp, improving the consistency of the pulp and flavoring it, coloring the pulp and converting it into paper, substantially as described.

9. The process of making wrappers from the fibrous portion of tobacco, which consists in separating the extractive and the cellular tissue from the fiber, converting the fiber into pulp, purifying the extractive, applying the purified extractive to the pulp, imparting an additional flavor to the pulp, and making the pulp into paper, substantially as described.

10. An improved tobacco wrapper, consisting of tobacco fiber deprived of its cellular tissue and other deleterious matter and treated to resemble the natural leaf.

11. An improved tobacco wrapper, consisting of paper obtained from tobacco fiber deprived of its cellular tissue and other deleterious matter and colored and treated to resemble the natural leaf.

12. An improved tobacco wrapper, consisting of paper obtained from tobacco fiber deprived of its cellular tissue and other deleterious matter, said paper being stained with tobacco-juice from which objectionable matter has been eliminated, and embossed to resemble the natural leaf.

13. An improved tobacco wrapper, consisting of tobacco fiber deprived of its cellular tissue and salts, and impregnated with tobacco-juice previously purified.

14. An improved tobacco wrapper, consisting of tobacco fiber deprived of its cellular tissue and other deleterious matter, flavored, and colored with tobacco-juice previously purified.

15. The process of making wrappers from tobacco stems and waste, which consists in separating the extractive and the cellular tissue from the fiber, converting the fiber into pulp, and treating the pulp to make it resemble natural leaf tobacco, substantially as described.

16. An improvement in the process of making wrappers from tobacco stems and waste, which consists in separating the extractive and cellular tissue from the fiber, converting the fiber into pulp, and imparting to the latter a tobacco flavor, substantially as described.

17. The process of making wrappers from tobacco stems and waste, which consists in separating the extractive and the cellular tissue from the fiber, converting the fiber into pulp, adding a percentage of licorice to the pulp, impregnating it with tobacco-juice of a high quality, and making the pulp into paper, substantially as described.

18. The process of making wrappers from tobacco stems and waste, which consists in separating the extractive matter and the cellular tissue from the fiber, making the fiber into pulp, improving the consistency of the pulp by the addition of glycerin, making the pulp into paper, and treating the paper to make it resemble natural-leaf tobacco.
19. The process of making wrappers from tobacco stems and waste, which consists in separating the extractive matter and the cellular tissue from the fiber, making the fiber into pulp, improving the consistency of the pulp by the addition of glycerin, purifying the extractive matter, applying the purified extractive matter to the pulp, imparting an additional flavor to the pulp, and making the pulp into paper.
20. The process of making wrappers from the fibrous portion of tobacco, which consists in separating the extractive matter and the cellular tissue from the fiber, making the fiber into pulp, adding glycerin to improve the consistency of the pulp, flavoring the pulp with licorice, impregnating the pulp with tobacco-juice of high quality, and making it into paper.
21. The process of making wrappers from the fibrous portion of tobacco which consists in separating the extractive matter and the cellular tissue from the fiber, making the fiber into pulp, adding glycerin to the pulp to improve its consistency, flavoring the pulp with licorice, purifying the extractive matter by elimination, applying the purified extractive matter to the pulp, and making the pulp into paper.
22. An improved tobacco wrapper consisting of tobacco-fiber paper deprived of its cellular tissue and extractive matter, and impregnated with extractive matter, which has been previously purified.
23. An improved tobacco wrapper consisting of tobacco-fiber paper deprived of its cellular tissue and extractive matter, and flavored with licorice, said paper being stained with extractive matter, which has been previously purified.
24. The process of making wrappers from the fibrous portion of tobacco, which consists in subjecting such portion to heat and moisture to extract a solution of soluble juice and salts and to loosen the fibers and cellular matter, straining and pressing the mass to separate the fibers from the cellular matter and from the solution of soluble matter, making the separated fibers into paper-pulp and treating the pulp to make it resemble the natural leaf.
25. The process of making wrappers from the fibrous portion of tobacco, which consists in subjecting such portion to heat and moisture to extract a solution of soluble juice and salts and to loosen the fibers and cellular matter, separating the fibers from the cellular matter, making the separated fibers into pulp, impregnating the pulp with a solution of purified extractive matter, and making the pulp into paper.
26. The process of making wrappers from the fibrous portion of tobacco, which consists in subjecting such portion to heat and moisture to extract a solution of soluble juice and salts and to loosen the fibers and cellular matter, separating the fibers from the cellular matter and pulping them, flavoring the pulp, making paper of the pulp, and thereafter treating the paper by staining and embossing it to make it resemble natural-leaf tobacco.
27. The process of making wrappers from the fibrous portion of tobacco, which consists in subjecting such portion to heat and moisture to extract a solution of soluble juice and salts and to loosen the fibers and the cellular matter, separating the fibers from the cellular matter and pulping them, adding glycerin and licorice to the pulp to strengthen and flavor it, purifying the extractive matter by elimination, impregnating the pulp with the extractive matter so purified, and forming the pulp into paper.
28. The process of making wrappers from the fibrous portion of tobacco, which consists in subjecting such portion to heat and moisture to extract a solution of soluble juice and salts and to loosen the fibers and cellular matter, straining and pressing the mass to separate the fibers from the cellular matter and from the solution of soluble matter, pulping the fibers, adding glycerin and licorice to the pulp to strengthen and flavor it, extracting cellular and deleterious matter from the solution, adding the purified solution to the pulp, and making the pulp into paper.
29. The process of making paper from the fibrous portions of tobacco, which consists in subjecting such portions in their natural condition to heat and moisture to extract a solution of soluble juice and salts and to loosen the fibers and cellular matter, separating the cellular tissue and extractive matter from the fibers, and then treating the fibers in the usual manner in paper manufacture.
30. The process of making wrappers from the fibrous portion of tobacco, which consists in subjecting such fibrous portion in an un-communited state, to heat and moisture to extract a solution of soluble juice and to loosen the fibers and cellular matter, separating the cellular tissue and extractive matter from the fibers, and then pulping and treating the liberated fibers in the usual manner in paper manufacture.
31. An improvement in the art of making wrappers from the fibrous portion of tobacco, which consists in separating the cellular tissue and extractive matter from the fibers before pulping the latter.
32. An improvement in the art of making

